

Patented Aug. 25, 1925.

1,550,912

## UNITED STATES PATENT OFFICE.

FREDERICK T. MANLEY, OF HOUSTON, TEXAS, ASSIGNOR TO THE TEXAS COMPANY, OF NEW YORK, N. Y., A CORPORATION OF TEXAS.

## LUBRICATING COMPOUND.

No Drawing.

Application filed October 1, 1920. Serial No. 414,083.

*To all whom it may concern:*

Be it known that I, FREDERICK T. MANLEY, a citizen of the United States, residing in Houston, in the county of Harris and State 5 of Texas, have invented certain new and useful Improvements in Lubricating Compounds, of which the following is a specification.

This invention relates to the preparation 10 of solid lubricants intended particularly for use in driving journals and for other heavy bearings working at high speed.

The invention contemplates the production 15 of a suitable lubricating compound that will be in the form of a cake or solid at ordinary temperatures but which will readily feed onto a bearing. It is an object of the invention to greatly reduce the cost of producing compounds of this nature by 20 utilizing certain cheap materials which have not hitherto been used in the manufacture of this type of lubricants. More specifically it is an object to use certain asphaltic products which not only reduce the cost of making the compound but add materially to the 25 lubricating value of the product.

In accordance with my invention I take a high boiling paraffin petroleum product such as a cylinder stock and mix it with 30 an asphaltic residue such as a viscous residue obtained from the distillation of Gulf Coast or other asphaltic base crudes. The compounded mineral oil is then mixed with a suitable soap such as soda soap to form a 35 solid lubricating compound. The proportions of cylinder stock and asphaltic residue may be varied somewhat according to the type of product desired but ordinarily the proportion consists substantially of 40 equal parts of each. The proportion of asphaltic residue may be increased to a certain extent but if too great a proportion of this material is used the product will tend to be friable and not suited for lubricating purposes.

45 As a specific example of my invention I may give the following:

Per cent.

|                              |       |
|------------------------------|-------|
| Fatty oil (e. g. tallow)     | 49.00 |
| Alkali (e. g. caustic soda)  | 9.04  |
| Water                        | 9.04  |
| Paraffin base cylinder stock | 16.26 |
| Asphaltic base residue       | 16.26 |
| Graphite                     | 00.4  |

It will be noted that in the example given a small quantity of graphite was included 55 in the compound but the graphite is not essential and may be omitted if desired. Any suitable soap may be used. For example, an alkali soap, such as soda soap, or a mixture of an alkali soap and lead soap, 60 may be employed in preparing the compound. It is understood that the mineral oil content and soap may be so proportioned as to give a mixture of the desired 65 degree of hardness.

The asphaltic base oil used may be any suitable asphaltic residue that has been reduced to the consistency of flux oil. It may contain greater or less proportions of oxidized oil and may be composed of asphalt 70 dissolved in an asphaltic base residue. The use of the oxidized oil seems to yield a product of exceptionally good lubricating value.

What I claim is:—

75

1. A solid lubricant comprising a soap, a paraffin base cylinder stock, and an asphaltic base residue.

2. A solid lubricant comprising a soap composition having for its mineral oil content substantially equal quantities of paraffin base cylinder stock and asphaltic base residue.

3. A solid lubricant comprising a soap, a paraffin base cylinder stock and asphalt 85 dissolved in an asphaltic base residuum.

4. A solid lubricant comprising in quantity approximately 50% fatty oil, 10% caustic soda, 10% water, 15% paraffin base cylinder stock, and 15% asphaltic base residuum.

5. A solid lubricant comprising in quantity approximately 50% fatty oil, 10% caustic soda, 10% water, 15% paraffin base cylinder stock, 15% asphaltic base residuum, 95 and a trace of graphite.

In witness whereof, I have hereunto set my hand this 17th day of September, 1920.

FREDERICK T. MANLEY.